

Patented Sept. 15, 1925.

1,553,758

# UNITED STATES PATENT OFFICE.

CARL FR. ECKERT, OF SAARBRUCK, GERMANY, ASSIGNOR TO ECKERT, OPPELT & CIE, GESELLSCHAFT MIT BESCHRANKTER HAFTUNG, OF SAARBRUCK, GERMANY, A FIRM.

## CORE FOR STEEL CASTINGS.

No Drawing.

Application filed November 14, 1922. Serial No. 600,954.

*To all whom it may concern:*

Be it known that I, CARL FRIEDRICH ECKERT, a citizen of the Republic of Germany, residing at Saarbruck, Germany, have 5 invented certain new and useful Improvements in Cores for Steel Castings, of which the following is a specification.

The invention relates to improved cores for smooth steel castings and more particularly for hollow steel castings such as ingot moulds, valve seatings, pump casings and the like. It is well known that the removal of the core from such castings offers considerable difficulties, as the mass from which 10 the core is made and which consists of chamot, quartzite sand and the like is found to have caked or baked. The removal of such cores from the casting can as a rule only be effected by the aid of pneumatic tools, which involves increased wages for 15 cleaning the castings. It has therefore already been suggested to obtain smooth castings by employing a special mould and core mass, the latter consisting essentially of ordinary sand with an admixture of loam or 20 of gypsum and fats or fatty oils or the like. For the manufacture of ordinary grey castings these cores are quite suitable, as grey iron is cast at a temperature of 25 1400-1500° according to quality. This mould and core mass can, however, not be employed for steel castings for the following 30 reasons: owing to the high temperature of the molten steel, which lies between 35 1700-1800°, the upper layer of the core melts at the moment when the steel is cast into the mould and sticks to the casting, forming a rough surface and a part of the core bakes together, owing to its low refractoriness, as even the best quartz sand 40 already sinters at a temperature of 1600°.

This invention consists of a core for steel castings in which the above named drawbacks and disadvantages are effectively 45 avoided.

The improved core consists either of an upper layer or entirely of aluminum-nitride or aluminum-nitride containing substances with the usual binding agents, for instance 50 molasses, tar and the like.

The core manufactured in this manner has the advantage that owing to its high refractoriness the core material does not burn to the casting and that the core after the 55 casting or after the burning of the binding

material does not cake at all and can be removed from the casting by the simplest tools or even by hand, as practical use has shown, without the least effort. From the hygienic point of view this must also be 60 considered of the greatest importance for the workmen engaged in cleaning the castings.

Experience has shown that the saving in wages for the cleaning of castings amounts 65 to about 70%.

A further advantage resides in the fact that the material of the improved core owing to its high refractoriness may be employed over and over again by simply replacing the 70 binding material.

In order to increase the strength of the core after the moulding or after the drying and to increase its porosity to enable gases to escape, the core may be further improved 75 by an addition of calcined clay or alumina.

The aluminum-nitride or the aluminum-nitride containing substances may also entirely be displaced by calcined clay.

The calcined clay is highly refractory and 80 quite free from injurious admixtures.

The advantages obtained by the employment of calcined clay consist in the greater firmness of the core, greater porosity and consequent easier escape of the gases and 85 easier removal of the core from the casting, than in the first described core.

What I claim as my invention and desire to secure by Letters Patent is:

1. As a new article of manufacture, the 90 improved core for producing hollow steel castings, consisting of an ordinary core covered with a coating containing aluminum-nitride mixed with a suitable binder.

2. As a new article of manufacture, the 95 improved core for producing hollow steel castings, consisting of aluminum-nitride mixed with a suitable binder.

3. As a new article of manufacture, the 100 improved core for producing hollow steel castings, consisting of an ordinary core coated with aluminum-nitride and calcined clay with a suitable binder.

4. As a new article of manufacture, the 105 improved core for producing hollow steel castings, consisting of a mass of material containing aluminum-nitride, and a suitable binder.

5. The process for producing cores for 110 steel castings, which consist in mixing a

coating containing aluminum-nitride with a suitable binding agent and covering an ordinary core with said coating.

6. The process for producing cores for 5 steel castings, which consists in mixing aluminum-nitride with a suitable binding agent and moulding the core thereof.

7. The process for producing cores for 10 steel castings, which consists in preparing a mixture of aluminum-nitride, calcined

clay and a suitable binding agent and coating an ordinary core therewith.

8. The process for producing cores for steel castings, which consists in preparing a mixture of aluminum-nitride, calcined clay 15 and a suitable binding agent and moulding the core thereof.

In testimony whereof I affix my signature.

CARL FR. ECKERT.